

Sept. 29, 1931.

A. S. HAMMOND

1,824,885

WAX PAPER

Filed Aug. 24, 1926



Inventor

*A.S. Hammond*

By his Attorneys

*Edwards, Tager and Brown*

## UNITED STATES PATENT OFFICE

ANNING SMITH HAMMOND, OF LOS ANGELES, CALIFORNIA, ASSIGNOR TO WESTERN  
WAXED PAPER COMPANY, OF OAKLAND, CALIFORNIA

## WAX PAPER

Application filed August 24, 1926. Serial No. 131,148.

This invention relates to an apparatus and method for making waxed paper and to the waxed paper product resulting from the method employed.

5 An object of this invention is to provide a waxed paper which will not "block" and will form a very efficient seal when heated. Broadly this object is attained by utilizing the advantages of different grades of wax 10 without their disadvantages while more specifically there is initially applied to the paper a wax having a relatively low melting point and then finally applied thereto a wax having a relatively high melting point.

15 A further object is to provide an improved apparatus and method for making waxed paper as above described.

Further objects and advantages will be apparent from the following description of the 20 accompanying drawing, which is a diagrammatic side elevation of the apparatus.

In the illustrative embodiment of the invention there is shown a receptacle 1, having compartments 2 and 3, separated by a suitable partition 4. Molten wax having a given 25 melting point will be disposed in compartment 2, while molten wax of a higher melting point will be contained in compartment 3. The wax in each case, such as paraffin or a 30 wax having similar qualities suitable for waxed paper of the self-sealing type wherein sealing of an article is accomplished by heat and pressure, is melted by suitable heating coils while the temperature thereof is con-

trolled by any suitable and usual temperature controlling mechanism. To wax a strip 35 of paper there is provided a suitably journaled roll of raw paper stock 5 from which a strip S will pass beneath an adjustable contact idler 6, and over the top of an advance roller 7, suitably journaled upon the top of the receptacle 1 so that the lower portion of the roller 7 will be immersed in the wax within compartment 2. The paper will continue 40

45 and pass over an adjustable scraper 8, then be completely submerged in the wax of compartment 3 by passing beneath an adjustable submerging bar 9, the paper continuing on between a steel roller 10 and a rubber roller 50 11, suitably journaled in the framework 12

after which it is led to suitable cooling rollers for final treatment and disposition.

It is to be noted that the wax in compartment 2 having the lowest melting point is applied preferably to only one side of the paper strip whereas the wax having a higher melting point is applied to both sides thereof. The scraper 8 removes any excess wax from the strip prior to its immersion in the wax within compartment 3.

By the method of first impregnating the raw paper with wax of a low melting point and then coating the paper with a higher melting point wax, I produce a waxed paper having an inner impregnated layer and an outer layer of wax, the outer one being a coating not readily affected by ordinary atmospheric temperatures but yet having qualities which permit an efficient seal to be made when heat and pressure are applied to the 70 wax paper, this being the characteristic of a wax having a high melting point when used in combination with the inner layer of impregnated wax having a lower melting point. On this account the wax will not soften 75 which, if it did, would permit the paper to stick together or "block" in warm weather. A further advantage obtained with such a coating is that the waxed paper will slide readily over metallic or wooden guide plates 80 usually employed in machinery such as automatic bread wrapping machines, which may become quite warm.

If a waxed paper contains only a wax of high melting point the same at ordinary temperatures will be brittle, but I have found that this disadvantage can be overcome by first applying the wax of lower melting point. The use of this wax not only overcomes any disadvantages of the higher melting point 90 wax, but has the further advantage because of its gumminess and tenacity at ordinary temperatures to supply a better sealing medium. Waxed paper to be sealed is usually heated under pressure, and under such conditions there will be a certain amount of admixture of the two kinds of wax, this occurring mostly at the surface of the paper at what might be called the "joint" of the two different waxes. As the gummy low melt- 100

ing point wax is available at this joint a better seal is obtained.

It will thus be seen that the apparatus employed permits the continuous passage of the paper strip through the various grades of wax without necessitating any interruption while at the same time the temperature of each grade of wax may be independently controlled. It will of course be understood that various modifications of such a machine could be had and that various auxiliary mechanisms that might be desired could be employed in connection with a machine such as diagrammatically disclosed herein. Any suitable mechanical drive could be employed for driving the necessary rollers for feeding the paper strips, such not having been shown in view of the nature of the drawing.

20 1 claim:—

1. The method of making self-sealing waxed paper consisting in first applying to a strip of paper wax having a given melting point and then applying a wax having a higher melting point.

25 2. The method of making self-sealing waxed paper consisting in first applying to one side of a strip of paper a wax having a given melting point and then applying a second coat of wax having a higher melting point.

30 3. The method of making self-sealing waxed paper consisting in first impregnating a strip of paper with wax having a low melting point by applying said wax to said strip on only one side thereof, and then applying to both sides of said strip wax having a higher melting point.

35 4. The method of making waxed paper consisting in first applying to a paper strip a wax having a low melting point, then applying wax having a high melting point, and then applying mechanical pressure to opposite sides of the strips.

40 5. The method of forming waxed paper consisting in taking a piece of raw paper stock and impregnating the same with a low melting point wax, then scraping the strip and then applying a final coating of wax having a higher melting point.

45 6. A wax paper of the type adapted to be sealed when overlapping portions thereof have heat and pressure applied thereto, consisting of paper stock having two coats of wax of different melting points.

50 7. A self-sealing wax paper consisting of paper stock having an inner coating of wax of a given melting point impregnated in the paper stock, and an outer coating of wax of a higher melting point whereby when pressure and heat is applied to overlapping portions of the waxed paper the two coatings of wax have some admixture so that the low melting point wax may permit its gummy qualities to become effective in sealing.

8. A wax sheet of paper consisting of paper stock impregnated with a low melting point wax, and an outer coating of wax on each side of the sheet, having a higher melting point.

9. The method of making waxed paper consisting in first impregnating a strip of paper with wax having a low melting point and then applying to both sides of said strip wax having a higher melting point.

ANNING SMITH HAMMOND.

75

80

85

90

95

100

105

110

115

120

125

130